

## UNITED STATES PATENT OFFICE

WILLIAM H. ADAMS, OF KENYON, RHODE ISLAND, ASSIGNOR TO EASTERN FINISHING WORKS, OF KENYON, RHODE ISLAND, A CORPORATION OF RHODE ISLAND

## MILDEWPROOF FABRIC AND PROCESS OF MAKING THE SAME

No Drawing.

Application filed September 4, 1929. Serial No. 390,419.

This invention relates to the treatment of fabrics made of cotton or other similar fibre for the purpose of rendering the same mildew proof. Cotton and other vegetable fibre 5 is destructively attacked by many forms of fungus growth of a vegetable nature, such as mildew, molds, dry rot, etc. These fungus growths belong to different groups and are so widely different in their nature that it has 10 been found to be impossible to provide a single protective agent which would protect the fibre or fabric against the action of all the different growths. Among the different groups of fungus growths referred to above 15 may be mentioned algae, growing in full light and in extreme wet surroundings. Fungus growths of this group are inhibited by water-soluble and water-decomposable salts of lead, copper, aluminum, zinc, mercury and some 20 more poisonous metals too dangerous to use.

A second group of fungus growth consists of mucors and similar molds usually growing best in damp and relatively dark surroundings and best inhibited by water-insoluble oxides of iron, chromium, manganese and cobalt. 25

A third group of such mildews includes the Aspergillæ and Penicillium varieties growing best under fairly light and only moderately damp conditions and best inhibited by water-insoluble compounds of chromium, lead, iron, cyanogen and in this class may be included the dry rots, whose growth is favored by relative darkness and poor ventilation. 30

As stated above these various groups and varieties of fungus growth are so widely different in their nature that it has been found to be impossible to provide a single protective agent which would protect the fibre or fabric against the action of all the different growths. Certain protective agencies will give protection against fungus growths of one type or group, other protective agencies 40 will give protection against fungus growths 45

of another type or group, etc., but if the several protective agencies are mixed together or are applied to the same surface of the fabric it has been found that they are apt to react on each other to such an extent as to 50 partially or wholly neutralize the protective capacity of each protective agent.

I have found, however, that by saturating the fabric or fibre with an aqueous solution containing ingredients antagonistic to one 55 main group of mildews and molds, such as that comprising the algae type and then drying the solution in place and subsequently coating successively the two faces of the fabric with two different kinds of water-proofing 60 mixtures containing in suspension two different mixtures of insoluble protective ingredients adapted to guard against or antagonize two other main groups of mildews or molds, I can produce a composite structure 65 which resists more completely all three groups of mildews or molds than would be done by the use of any single combination. The first applied water-soluble compound even after 70 drying is not removed by the two subsequent volatile solvent mixtures carrying inhibiting 75 solids in suspension, and though sufficiently impermeable to prevent these latter applications from mixing injuriously do not prevent their mildew inhibitory characters from manifesting themselves, and these latter applications tend to water-proof and protect from leaching or soaking the first applied water-soluble mixture or compound.

Furthermore, if the first protective agent 80 is of such a character that the protective ingredients therein are relatively insoluble in or impermeable by the materials with which the faces of the fabric are coated then the first-named material with which the fabric is 85 saturated forms a barrier between the two surface coatings and prevents them from mingling in such a way as to neutralize each other to any degree without preventing their mildew inhibiting activity. 90

In carrying out my invention I propose first to treat the fabric or fibre by saturating it in an aqueous solution containing water soluble compounds of lead, copper, aluminum, zinc, mercury or other metals capable of being fixed by drying and repellent or poisonous to a specific group of mildews or molds. The fabric or fibre thus saturated is then dried and subsequently one side of the 10 fabric is coated with a non-aqueous waterproofing liquid adapted to combat a second and different group of mildews and moulds. This waterproofing liquid may consist of waterproofing waxes, gums, resins, greases or 15 oils melted or dissolved in a volatile solvent and carrying in suspension finely divided solid matter, such as a compound of chromium, lead and iron and cyanogen which may or may not be suitably diluted with finely 20 divided solid inert matter. The other face of the fabric is then coated with another solution of waterproofing materials which are adapted to resist and antagonize a third group of mildews or molds different from 25 the other two groups.

Such waterproofing material may consist of similar waxes, gums, resins, oils or greases dissolved in a volatile solvent and carrying in suspension finely divided insoluble solid 30 matter consisting of iron oxides, iron and manganese oxides, or a compound of iron manganese and cobalt oxides suitably diluted with finely powdered inert solid matter.

As illustrative of some protective agencies 35 coming within the scope of the invention I would refer to the following.

One suitable solution for saturating the fabric in the first instance and which solution is antagonistic to one group of mildews or 40 molds may be made according to the following formula, which for convenience I will refer to as "Formula A."

#### Formula A

|                              | Pounds |
|------------------------------|--------|
| 45 Basic lead acetate        | 10     |
| Copper acetate               | 2      |
| Aluminum acetate (strong)    | 10     |
| Mercuric chloride or acetate | 1      |

50 These ingredients are dissolved in cold water and diluted to a specific gravity of from 5° to 12° Twaddel.

Another suitable solution for this purpose 55 may be made according to the following formula, which for convenience is referred to as "Formula B."

#### Formula B

|                           | Pounds |
|---------------------------|--------|
| Lead acetate              | 10     |
| 60 Copper acetate         | 2      |
| Aluminum acetate (strong) | 10     |
| Zinc acetate              | 1      |

The above is dissolved in cold water and 65 diluted to a specific gravity of from 5° to 12° Twaddel.

A suitable protective agent adapted to be applied to one surface of the fabric and which is antagonistic to another group of mildews or molds may be made according to the following formula, which for convenience 70 I will refer to as "Formula C".

#### Formula C

|                          | Pounds |
|--------------------------|--------|
| Cold-vulcanized corn oil | 10     |
| Paraffin wax             | 15     |
| Beeswax                  | 15     |
| Ceresin                  | 15     |
| Carnauba wax             | 5      |
| Linseed oil              | 10     |
| Petrolatum               | 20     |

The above is dissolved in from 20 to 30 gallons of naphtha according to the thickness of coating desired and the following ingredients are then incorporated in the solution: 85

|                                     | Pounds |
|-------------------------------------|--------|
| Finely powdered dry iron oxide      | 16     |
| Finely powdered dry manganese brown | 3      |
| Cobalt oxide                        | 1      |

Another protective agent which may be used in place of the above may be made according to the following formula, which for convenience I will refer to as "Formula D".

#### Formula D

|              | Pounds |
|--------------|--------|
| Paraffin wax | 40     |
| Ceresin wax  | 10     |
| Beeswax      | 10     |
| Carnauba wax | 3      |
| Petrolatum   | 100    |

The above ingredients are melted together and then 16 lbs. of finely powdered dry iron oxide, 3 lbs. of finely powdered manganese oxide are added to the solution. 105

A suitable protective agent for coating the other side of the fabric and which is antagonistic to still another group of mildews or molds may be made according to the following formula, which for convenience I will refer to as "Formula E". 110

#### Formula E

|                          | Pounds |
|--------------------------|--------|
| Cold-vulcanized corn oil | 10     |
| Ceresin                  | 15     |
| Japan wax                | 15     |
| Paraffin wax             | 15     |
| Beeswax                  | 10     |
| Carnauba wax             | 5      |
| Linseed oil              | 10     |
| Petrolatum               | 20     |

The above is dissolved in 20 to 30 gallons of naphtha and then has incorporated therein 125 12 pounds of finely powdered lead chromate (dry); 9 pounds finely powdered ferric ferrocyanide (dry); 12 pounds finely powdered steatite or asbestine (dry).

Still another formula by which an equivalent material may be made is as follows, 130

which for convenience I will refer to as "Formula F".

*Formula F*

|                     | Pounds |
|---------------------|--------|
| 5 Paraffin wax----- | 40     |
| Ceresin wax-----    | 10     |
| Beeswax-----        | 3      |
| Petrolatum-----     | 20     |

10 The above are melted together and then have incorporated therein

|                                                   | Pounds |
|---------------------------------------------------|--------|
| Finely powdered dry lead chromate-----            | 7      |
| Finely powdered dry ferric ferrocyanide-----      | 5      |
| 15 Finely powdered dry asbestine or steatite----- | 5      |

20 The above formulae are not intended to cover all of the different protective agencies which fall within my invention but are only mentioned as giving examples or illustrations.

The solutions made according to Formulae A and B provide the fabric with ingredients which are impermeable by the ingredients of the other formulae. The aqueous protective 25 agencies or coatings applied to opposite sides of the fabric are of such a nature that if they were brought together in solution they would react in such a way that each would partially neutralize the mildew-repelling effect of the 30 other, but by first saturating the fabric with a water-soluble protective agent such as described in either Formula A or B, the ingredients of which are impermeable by the 35 ingredients of the agents that are applied to the surfaces of the fabric, the water-soluble material with which the fabric is saturated forms a barrier between the two surface layers that prevents them from coming into contact and thus neutralizing each other while 40 at the same time the non-water soluble surface layers act to waterproof and protect the water-soluble materials with which the body and center of the fabric are saturated.

The fabric is thus provided with the three 45 different protective agencies, each of which is adapted to combat or antagonize mildews or molds of some particular group and these three protective agencies are so applied that no one of them affects the protective action 50 of any of the others so that when treated according to my invention the fabric receives the full benefit of all three of the different protective agencies.

I claim.

55 1. A mildewproof fabric comprising a fabric saturated with a mildew-resistant agent which is repellent to mildews of one group, said fabric having on each face a superficially applied mildew-resistant agent which is repellent to mildews of a particular individual group, the mildew-resistant agents which are superficially applied to the faces of the fabric having the capacity of neutralizing each other when brought into contact and the 60 protective agent with which the fabric is sat-

urated being impermeable to the other mildew-resistant agents and constituting a barrier between them which prevents them from reacting on each other.

2. A mildewproof fabric comprising a fabric saturated with a mildew-repellent agent containing a metal acetate, each surface of the fabric being coated with a mildew-repellent agent containing waxes and metal oxide. 70

3. A mildewproof fabric comprising a fabric saturated with a mildew-repellent agent containing metal acetate and which is repellent to mildews of one group, each face of the fabric being coated with a different mildew-repellent agent repellent to its own individual group of mildews, the first-named agent with which the fabric is saturated constituting a barrier between the other two agents which prevents them from reacting on each other. 75

4. A mildewproof fabric comprising a fabric saturated with a mildew-repellent agent containing metal acetate and which is repellent to mildews of one group, each face of the fabric being coated with a different mildew-repellent agent repellent to its own individual group of mildews, the mildew-repellent agent with which the fabric is saturated being impermeable by the other mildew-repellent agents. 80

5. The method of mildewproofing a fabric which consists in saturating the fabric with a mildew-repellent agent repellent to mildews of one group, applying to one face of the fabric a different mildew-repellent agent which is repellent to mildews of a second group and which will not permeate the first-named mildew-repellent agent and then coating the other face of the fabric with a third mildew-repellent agent repellent to a still different group of mildews. 85

6. The process of mildewproofing fabric which consists in saturating the fabric with a water solvent mildew repellent agent, drying the protective agent in place, and then coating the two faces of the fabric with two different volatile solvent mildewproofing waterproofing solutions, neither of which will permeate the agent with which the fabric is saturated. 90

In testimony whereof, I have signed my name to this specification.

WILLIAM H. ADAMS.

120

125

130